

# United States Patent Office

2,719,797

Patented Oct. 4, 1955

1

2,719,797

## PLATINIZING TANTALUM

Edgar F. Rosenblatt, Montclair, and Johann G. Cohn, East Orange, N. J., assignors to Baker & Co., Inc., Newark, N. J., a corporation of New Jersey

No Drawing. Application May 23, 1950,  
Serial No. 163,782

13 Claims. (Cl. 117—65)

This invention relates generally to a process for coating tantalum and like metals with metals or alloys of the platinum group and is furthermore concerned with improved anodes manufactured according to this coating process. The invention also relates to the application of these improved anodes in certain electrochemical reactions and it relates particularly to a process to produce platinized tantalum for use as non-corroding anodes in electrochemical processes.

In electrochemical processes, such as the electrolysis of chlorides and the production of percompounds, the proper selection of material from which to manufacture the electrodes is a matter of prime importance. In these processes, it is conventional to use electrodes of iron, steel, etc., in the cathode position; however, there are only a few known materials that may constitute the anodes, because most materials while in the anode position are susceptible to intense corrosion. If only the chemical characteristics of a material were to be considered in the selection of a suitable anodic material, the metals of the platinum group would be the universal choice because they are highly resistant to corrosion; however, the high cost of these precious metals prohibits their extended commercial use. Substitute materials have, therefore, been resorted to, whenever possible, the primary anodic material employed industrially being that of graphite.

Many disadvantages accompany the use of graphite as an anodic material. A graphite anode undergoes continual disintegration and must be replaced from time to time thereby causing interruption of the electrochemical process which is a costly operation. In the manufacture of chlorine by the electrolysis of brine, it is necessary to purify the product from traces of carbon dioxide which result from the oxidation of the graphite anodes. Particles which dust off from the graphite become deposited in the diaphragms which surround the electrodes thereby necessitating replacement of the diaphragms along with the electrodes. These difficulties are not encountered when anodes of the platinum metals are used. Also the over-voltage characteristics for chlorine discharge are more favorable with platinum metal anodes than with graphite anodes.

There has been a continual search for a material which has the desirable anodic characteristics of the platinum metals, but not their prohibitive costs. It has long been considered that tantalum would make an ideal anodic material because of its remarkable chemical inertness. Tantalum is not attacked by chlorine, hydrochloric acid, nitric acid, or aqua regia. Then, too, its cost is very low as compared with the cost of the platinum metals. However, when a tantalum electrode is used as an anode, the flow of electric current through the cell quickly stops. This phenomenon is caused by the formation of what may be referred to as an anodic film comprising a layer of oxide which decreases the electric conductivity of the material.

In order to prevent the formation of this film, attempts have been made to coat a tantalum base with platinum

2

metal. It has been suggested that coating with a platinum metal be accomplished by such methods as electrolysis, hammering, welding, rolling, and the like; however, none of these methods have been found to be satisfactory. 5 They do not produce a coat of platinum metal which adheres with sufficient tenacity to the tantalum base that the coated tantalum metal will be commercially suited for use as an anode in electrochemical processes. Electroplating of a platinum metal onto a tantalum base results 10 in a coating that may easily be stripped from the base. Attempts to cover the tantalum strip with a platinum metal foil and to hold the metals together as by sweating, rolling or hammering, have proved to be unsatisfactory because the platinum metal foil is held to the tantalum 15 only by mechanical contact which is not sufficient to permit of its use as an anode. The coats of platinum metal that have been made by any of these processes are not truly bonded to the tantalum, i. e. the tantalum is not platinized in the sense that the platinum metal is united 20 with the tantalum by atomic attraction forces as is obtained by this invention.

It is, therefore, one object of this invention to provide a thin, firmly adherent, practically inseparable coat of one or several of the platinum metals onto a base of tantalum or like metal. It is a further object of the invention to achieve this result in a simple and economical manner. Another object of this invention is to manufacture a composite metal stock having a bodily new arrangement between tantalum and platinum metals. It is a further object of this invention to improve certain electrochemical processes by using the improved electrodes of this invention. Further objects and various advantages of this invention will become apparent from a consideration of this specification and the appended claims.

35 By the term "platinum metal," as herein used, is meant the precious metals in group VIII of the periodic chart, excepting osmium, i. e. this term includes the following metals: ruthenium, rhodium, palladium, iridium and platinum.

40 Broadly, the process of this invention involves a combination of successive treatments whereby a thin deposit of a platinum metal is made upon the surface of a tantalum body and thereafter the platinum metal deposit is bonded to the tantalum body by heating the whole to a high temperature and under inert conditions. The thin deposit of a platinum metal may be applied according to this invention in one of several different ways, such as by electroplating or by the chemical decomposition of a platinum metal compound applied on the surface of the tantalum. It should be clearly understood that the thin deposits made according to any of these processes are not firm deposits until they have been subsequently bonded in the manner described later in this specification.

45 For the purpose of this invention, columbium may be used instead of tantalum. Also, alloys, including sintered products of these metals, may be used, i. e. alloys of the metals themselves as well as with the addition of other metals which do not change the inertness of the alloy. At the present time, tantalum is preferred over 50 the use of columbium because the cost of columbium is much greater than the cost of tantalum. It is intended also that the term "tantalum" as used herein be not limited to the chemically pure metal but that it include the marketable form which contains small and, therefore, harmless traces of impurities, such as carbon, iron, etc.

### Chemical decomposition

55 As stated above, one method of applying a thin coat of a platinum metal is by decomposing a metal compound on the surface of the tantalum. To accomplish this treatment, the tantalum base is preferably washed as with

carbon tetrachloride and acetone. The surface of the tantalum metal is then cleaned and roughened to an extent depending upon the amount of coverage that is desired. This roughening may be accomplished by rubbing the metal with emory papers, by sand blasting, or by chemically etching with hydrofluoric acid. The etching may also be accomplished electrolytically in hydrofluoric acid using lead or silver as the cathode material. The cleaned and roughened tantalum is then dipped into or otherwise coated with a solution of, e. g. chloroplatinic acid ( $H_2PtCl_6$ ), which has been dissolved in a suitable volatile solvent. It has been found that one gram of chloroplatinic acid dissolved in a solution containing 15 ml. isopropyl alcohol and 15 ml. ethyl acetoacetate produces a uniform platinum coating. The more important constituent of this solvent is the ethyl acetoacetate since solutions having a higher concentration of this constituent give better results than do those having a greater proportion of the alcohol. After dipping the tantalum into this solution, the excess solution is removed and the solvent is evaporated off at a relatively slow temperature. The coated tantalum is then heated above the decomposition temperature (approximately 250° C.) of the chloroplatinic acid whereby a thin coat of platinum is left upon the tantalum surface, all other products of the decomposition being volatile. The platinum coating resulting from the above treatment amounts to approximately 0.00034 gram/cm.<sup>2</sup>. In like manner, tantalum and columbium may be coated with other metals of the platinum metal group by using one of the following chemical compounds ruthenium nitroso bromide



palladium di-n-butylamine nitrite



and iridium chloride acid ( $H_2IrCl_6H_2O$ ).

#### Electroplating

Another method for depositing the thin coat of a platinum metal upon the tantalum base is by electrolysis. After the tantalum base has been roughened as by etching in a manner as explained above, it is placed in the cathode position in a plating bath. A plating bath having the following composition has been found to be suitable:

20 g.  $Pt(NH_3)_2(NO_2)_2$  commercially known as P-salt  
100 g. ammonium nitrate  
1 liter of 5% ammonia

The temperature of the bath is maintained at approximately 90–93° C. and it is constantly stirred. Neither the concentration of the P-salt, nor that of ammonia is critical. Even heavy platinum deposits may be plated out from this bath with unchanged current efficiency. The ammonia which evaporates rapidly at elevated temperatures may be replaced arbitrarily by keeping the bath smelling. The P-salt must be replenished from time to time by adding solid salt corresponding to the amounts of platinum plated out.

#### Bonding

Following the deposition of the thin platinum metal coating, the coated tantalum is subjected to the bonding treatment of this invention. An example of the manner in which this treatment is carried out follows:

Tantalum strips which have been platinized according to the above described chemical decomposition or electroplating procedures are placed into a cold furnace. The furnace is evacuated to about  $10^{-4}$  mm. of mercury and is then heated to a temperature below the lowest melting point of the metals involved and high enough to cause the metals to become bonded as required by this invention. Temperatures ranging from approximately 800° C. to 1400° C. have been found suitable, the op-

timum temperature being about 1000° C. After the bonding temperature has been maintained for approximately 15 minutes, the heating is discontinued, and when the temperature in the furnace has substantially dropped the evacuation is stopped and the coated tantalum is removed. Instead of treating the metal in a vacuum, it has been found that any inert atmosphere such as helium, neon, argon, and the like may be substituted. These gases do not chemically combine with the tantalum as does oxygen, for example, and by the term "inert conditions" as used in this specification and in the claims is meant such surroundings which are inert with respect to tantalum, such as a vacuum or a noble-gas atmosphere.

A platinum layer on a tantalum strip which has not been subjected to the bonding treatment of this invention will upon being immersed in aqua regia become completely dissolved. When, however, such a coated strip is bonded in the manner described above, aqua regia will not completely dissolve the platinum layer and the weight of the bonded strip after it has been immersed in aqua regia is greater than the weight of its original tantalum constituent, thus indicating that the bonding treatment causes the platinum and tantalum metals to interdiffuse and become alloyed in such a composition that the alloy is not attacked by hot aqua regia.

Tantalum strips which were platinized by the above described chemical decomposition procedure were heated in vacuum at 1200° C. and 1400° C. Platinizing according to this procedure produces layers of only up to 0.03 mm. in thickness per application. The layers thus deposited were not attacked by hot aqua regia, however, when these strips were tested as anodes in cells for the production of chlorine and chlorates the current ceased to flow and the strips became corroded with a coherent tarnish layer. This corrosion of the anode indicates that the tantalum metal has diffused through the thin platinum layer to the outside surface of the platinum film where the tantalum becomes oxidized and stops the flow of current through the cell. If platinized tantalum strips are bonded at temperatures of less than 800° C., the platinum metal layer is easily dissolved by aqua regia and the platinum films flake off from the tantalum base when the strips are used as anodes, thus indicating that substantially no alloying of the platinum and tantalum metals occurs when there is insufficient heating.

It is desirable, therefore, to coat the tantalum base in such a manner that the outside layer of the platinum metal film will consist of substantially pure platinum whereas the inside layer of the film will be firmly bonded to the tantalum base by the formation of a thin layer of platinum-tantalum alloy. A tantalum strip which has been platinized in such a desired manner will behave like an ordinary platinum electrode, the apparently vulnerable zone of platinum-tantalum alloy being protected from contact with the electrolyte solution in the cell by the outer layer of unalloyed platinum. To insure that the outer layer remains unalloyed during the heat treatment by which tantalum and platinum become bonded, a heavier platinum metal coat is required than in the alloy anodes described above. Also from a commercial standpoint, it is advantageous to apply a relatively thick platinum metal coat on a thick tantalum base and, thereafter, roll or otherwise draw out the thick coated bar to obtain the desired reduced strips having a top layer of unalloyed platinum metal. Such a procedure permits of more ease in the handling of the metal composites and enables using smaller processing equipment having obvious economical advantages as well as reducing the losses incurred during the etching treatment.

A heavy deposit of platinum metal may be applied to the tantalum base by electroplating in the manner described above; however, if such heavy deposit exceeds approximately 1 mu. in thickness, it cannot be successfully bonded. Apparently, during the electroplating process, stresses are generated in the platinum film caus-

ing blisters to form which do not become coherently bonded to the tantalum base when the coated metal is subsequently heated.

In practicing this invention, it is, therefore, desirable to apply a primary coat which does not exceed 1 mu. in thickness. Following the bonding of the primary coat to the tantalum base in the manner as hereinabove described, a second coat of any desired thickness, such as for example 25 mu., may be electroplated upon the surface of the thin primary coat. The blistering which occurs as stated above when a thick platinum metal deposit is electroplated directly upon a tantalum base, does not occur when the second coat is deposited.

Following such a procedure, it has been found possible, for example, to platinize a tantalum rod of 6.7 millimeters diameter with a platinum film of 25 microns in thickness, and, thereafter, to draw out the coated and bonded rod to a diameter of .67 millimeter without any danger of splitting the platinum film from the tantalum base. This rod after being reduced in diameter behaves like a pure platinum anode thus indicating that the platinum-tantalum alloy which is formed at the interface of the film and the base does not extend to the outside surface of the film, and that the outer surface layer of the film comprises substantially pure platinum. Also, there is no flaking off of the platinum film even after long and continued use of the rod as an anode in a chlorine or chlorate production cell, thus indicating that the platinum film is firmly bonded to the tantalum base.

The secondary coat may be applied in several separate layers and between the periods of the deposition of these several layers, the metals may be subjected to a bonding treatment. It is preferred that the primary coat be not more than 5% of the thickness of the secondary coat or the combined layers which may comprise the secondary coat.

It has been furthermore observed that the original surface film of the tantalum body that is not removed by the cleaning and roughening process, becomes diffused throughout the interior of the tantalum mass during the subsequent heating treatments whereby pure tantalum metal becomes joined by atomic attraction forces with the platinum deposit. When, however, no precautions are taken to prevent the formation of the surface film during the heating treatments, the film becomes considerable and is not completely dissolved into the tantalum mass, thus preventing the platinum deposit from joining directly to the pure tantalum. Also, it is noted that the diffusion of this surface film into the tantalum mass causes the development of permanent hardness of the tantalum, and when relatively large amounts of oxygen or nitrogen are absorbed in the metal, the tantalum becomes brittle. This brittleness is especially pronounced in the case where very thin strips of tantalum are used. By depositing platinum metals and bonding them to tantalum according to the process of this invention, these undesirable results are eliminated.

Examination with a microscope of the platinum metal films of this invention reveals that they have a rough or wavy profile, the indentations of which develop into pores when the coated sheets are reduced to small thicknesses. Although these pores expose the tantalum to the development of an anodic film, the coated tantalum spots are not affected when the composite metal is used as an anode. Also, the thin platinum outer layer prevents the alloy layer from being attacked.

The inner core of the tantalum base may consist of copper, silver, or other like metal. For example, a tantalum tube which has been platinized on its outer surface according to the method of this invention may be slipped over a tightly fitting copper rod and the composite rod may then be swaged and drawn to any desired thickness. When using such a composite rod as an anode in the electrolytic production of chlorine, chlorates, and per-compounds, it is necessary that the tantalum covering

have no openings through which the core metal may be attacked.

From the above description, it will be seen that we have disclosed a process by which platinum metals may be successfully and firmly bonded to tantalum metals, and that tantalum which has been platinized according to the manner taught herein may be used as an anode in electrochemical processes, and especially in the production of chlorine, chlorates, and per-compounds. The examples which have been included in this specification have been given by way of illustration only and not by way of restriction or limitation. We desire to have it understood that we do not intend to limit ourselves to the particular details described except as defined in the claims.

What we claim is:

1. A method of providing an adherent coating of platinum metal on a base of material of the group consisting of tantalum and columbium, comprising the sequential manufacturing steps of depositing a thin continuous layer of platinum metal on said base and heating said layer and said base in proximity thereto under inert conditions at an elevated temperature below the melting point of said platinum metal and said base material and within the range of about 800° C. to about 1400° C. to inter-diffuse said metals at the boundary thereof, whereby said platinum metal layer becomes bonded to said material on its outer surface and is separated from the base by an interlayer of an alloy of the platinum with the base metal.

2. A method of coating a base formed of material selected from the group consisting of tantalum, columbium and alloys of these metals platinum metal comprising the sequential manufacturing steps of depositing a primary coat of platinum metal on said base heating the coated base under inert conditions at an elevated temperature within the range of about 800° C. to about 1400° C. the melting point of said metals to alloy the adjacent surfaces of said metals, electroplating a second coat of platinum metal on said primary coat, and heating the coated mass at an elevated temperature below the melting point of said metals and within the range of about 800° C. to about 1400° C. to form coatings of pure Pt interspersed with interlayers of an alloy of Pt with the base metal.

3. The method according to claim 2 wherein said second coat comprises a plurality of separate deposited layers and the composite metal is subjected to the step of heating under inert conditions below the melting point of said metals and within the range of about 800° C. to about 1400° C. to alloy the adjacent surfaces of said metals between the steps of applying each separate layer deposit.

4. The method according to claim 2 wherein the thickness of the primary coat is not more than 5 percent of the thickness of the second coat.

5. A method of producing an anode for use in electrochemical processes by providing an adherent coating of platinum metal on a base of tantalum which comprises the sequential manufacturing steps of cleaning and roughening the surface of the tantalum, depositing a thin first coat of platinum metal on the tantalum base, bonding said coat to said base by heating said metals in an inert atmosphere at a temperature above about 800° C. but below about 1400° C. whereby the remaining film migrates into the metals and the adjacent surfaces of said layer and said base are alloyed and said metals are joined together by atomic attraction forces, electroplating a second coat of platinum metal upon said first coat, heating the metals to an elevated temperature within the range of about 800° C. to about 1400° C., and reducing the thickness of the bonded metals.

6. The method according to claim 5 wherein the cleaning step is performed by etching the tantalum with hydro-

fluoric acid, the inert atmosphere being a vacuum, and the bonding temperature being about 1000° C.

7. The method according to claim 5 wherein said second coat comprises a plurality of separate deposited layers and the base and deposited layers are subjected to the step of heating under inert conditions below the melting point of said metals and within the range of about 800° C. to about 1400° C. to alloy the adjacent surfaces of said metals between the steps of applying each separate layer deposit, the thickness of said first layer being less than about 5 percent of the thickness of said second coat.

8. The method according to claim 1 wherein the step of depositing the layer of platinum is accomplished by washing said base metal with a solvent, cleaning and roughening said base metal as by etching, coating said cleaned base metal with a solution comprising a soluble compound of the platinum metal and a volatile solvent, evaporating the solvent from the liquid, and heating the coated base metal above the decomposition temperature of the soluble compound to decompose said compound and to volatilize the products of decomposition excepting the platinum metal.

9. The method of claim 8 wherein the soluble compound is chloroplatinic acid and the solvent is a mixture of isopropyl alcohol and ethyl acetoacetate.

10. The method according to claim 1 wherein the step of depositing the layer of platinum is accomplished by electrolysis.

11. The method of claim 2 wherein the primary coat

5 is deposited by washing said base metal with a solvent, cleaning and roughening said base metal by etching, coating said cleaned base metal with a solution comprising a soluble compound of the platinum metal and a volatile solvent, evaporating the solvent from the liquid, and heating the coated base metal above the decomposition temperature of the soluble compound to decompose said compound and to volatilize the products of decomposition excepting the platinum metal.

10 12. The method of claim 11 wherein the soluble compound is chloroplatinic acid and the solvent is a mixture of isopropyl alcohol and ethyl acetoacetate.

15 13. The method of claim 2 wherein the primary coat is deposited by electrolysis.

References Cited in the file of this patent

UNITED STATES PATENTS

|           |            |               |
|-----------|------------|---------------|
| 1,465,553 | Kirk       | Aug. 21, 1923 |
| 2,114,161 | Antisell   | Apr. 12, 1938 |
| 2,226,720 | Hansell    | Dec. 31, 1940 |
| 2,282,097 | Taylor     | May 5, 1942   |
| 2,303,497 | Reeve      | Dec. 1, 1942  |
| 2,370,242 | Hensel     | Feb. 27, 1945 |
| 2,375,154 | Volterra   | May 1, 1945   |
| 2,401,040 | Becker     | May 28, 1946  |
| 2,417,459 | Eitel      | Mar. 18, 1947 |
| 2,418,460 | Buehler    | Apr. 8, 1947  |
| 2,492,204 | Van Gilder | Dec. 27, 1949 |
| 2,497,109 | Williams   | Feb. 14, 1950 |
| 2,539,096 | Miller     | Jan. 23, 1951 |